

## UNITED STATES PATENT OFFICE

1,925,627

## MANUFACTURE OF BLEACHING POWDER

Charles Carter, Hunts Cross, Liverpool, England, assignor to Imperial Chemical Industries Limited, London, England, a British company

No Drawing. Application November 17, 1930,  
Serial No. 496,332, and in Great Britain  
November 26, 1929

## 5 Claims. (Cl. 23—86)

This invention relates to an improvement in the process of manufacturing bleaching powder (either ordinary or the socalled tropical bleaching powder) by interaction of partially or wholly slaked lime or partially chlorinated lime with a counter current of diluted chlorine in an agitating apparatus, adapted for continuous production. The conditions here are quite different from those of processes such as the Weldon chamber process, in which strong chlorine is used without agitation of the solid in counter current and my invention relates to continuous processes of the type set forth.

It is well known that bleaching powder is conveniently prepared by agitation of slaked lime in counter current to chlorine gas diluted with more or less air, preferably in a rotary tube. Hitherto the output of any particular rotary tube has been limited, not only by the speed of the reaction, which normally requires of the order of 8 hours contact between lime and chlorine, but by the rate of dispersal of heat. The only means of dispersal of heat have been, so far, heat radiation or external cooling, and circulation of a large volume of air which may or may not be refrigerated before entering the plant, and which leaves the plant at an elevated temperature. Heat is also absorbed in the evaporation of part of the water liberated in the reaction. Up to now any attempt to increase the output to any considerable extent has resulted in weak bleaching powder.

In view of the desirability of ultimately producing a product low in moisture, it has hitherto been the tendency to exclude moisture as far as possible and it has been proposed to dry the circulating air.

I attribute the failure to produce until now strong bleach on increased output not only to decomposition, caused by excessive temperature, but also to premature drying of the partly chlorinated lime to such a stage that further chlorination, if it proceeds at all, is extremely slow.

I have now found that it is possible to produce full strength bleaching powder very rapidly in an agitating apparatus, by introducing water into the apparatus during the operation. The water so introduced prevents the premature drying above referred to thus permitting the reaction to take place in a very short time, and enabling a larger output to be obtained in any particular rotary tube. An important feature of the invention consists in distributing in the apparatus liquid water which, by its evaporation, functions as a very efficient cooling agent and also secures

the further benefits referred to above. The water is preferably introduced in an "atomized" condition, by means of any suitable spray, which protrudes into a rotary tube or other agitating apparatus and delivers the water preferably at 60 the zone of greatest reaction. The quantity of water used will be adjusted according to, among other conditions, the output desired, the volume of circulated gas, and the proportion of water desired in the resulting bleaching powder. The 65 water spray has the additional advantage that it reduces the quantity of dust carried off in the exit gases.

When using liquid water, I may employ slaked or partially slaked lime or partially chlorinated 70 lime.

As examples of the quantities of water required to be used I give the following.

1. In a cast iron rotary tube of dimensions 20 ft. by 3 ft. capable normally of an output of less 75 than 1 ton per day I have obtained an output of 2.6 tons bleaching powder per day by spraying in water at the rate of .23 tons per day.

2. In the same rotary tube an output of 4 tons bleaching powder per day was obtained by spraying in .68 tons of water per day.

3. In a 60 ft. cylinder capable normally of an output of 4 to 5 tons bleaching powder per day from already partly chlorinated lime averaging 8 to 10% available chlorine, the output was increased to 8 to 10 tons per day by spraying in water at a rate of about .3 tons water per day, the lime feed, the speed of the cylinder, and the chlorine and airflow being doubled.

Needless to say I do not confine myself to these 90 examples. As mentioned above, the quantity of water used will depend on many other conditions. As seen from the above examples even the proportion of water to lime will not be constant, since it will vary with different designs of plant, and will, for any particular plant, increase as the output is increased, and will also depend to some extent on the atmospheric temperature and on the temperature of the input gases. In general it will be adjusted as explained in my broad outline of 95 principle given above, so that the quantity of water evaporated absorbs in its evaporation the surplus heat, thus preventing premature drying and excessive temperature.

Some of the advantages of the invention can 100 be obtained by use of high moisture lime, that is to say lime which contains a higher proportion of water than corresponds to that of calcium hydrate, but I prefer the introduction of liquid water 105 which controls the temperature, accelerates the

reaction and reduces the amount of dust carried off.

The use of liquid water is preferred, steam being very much less efficient for my purpose since it exerts no cooling action such as that resulting from the evaporation of sprayed liquid water.

The use of high moisture lime suffers from certain disadvantages chief amongst them being the difficulty of feeding it mechanically at a uniform rate.

According to a further modification of the present invention I treat slaked lime or partially chlorinated lime with hot gases containing chlorine whilst adding water to prevent premature drying of the material. In this way it is possible to produce directly a high-strength bleaching powder suitable for use in tropical countries (e.g. a product containing say 1 to 1½% only of moisture).

It has been proposed to produce the so-called tropical bleaching powder by drying previously made bleaching powder with hot air in a second operation (British Patent 242,805) or by direct production of one operation, using circulation of a large volume of dilute chlorine which, assisted by the heat of reaction, allows of removal of moisture by the circulating gas.

I have attempted to use hot inlet gases for the purpose of effecting chlorination and drying in one operation but the resultant product was weak, if properly dried. I believe this result is due to premature drying of the bleach. My present invention allows me to obtain the advantage of using hot inlet gas and yet by injecting water into the apparatus (which may be a rotary tube) I avoid this premature drying and thus secure thorough chlorination of the solid, which as it proceeds along the tube is dried by the hot gas. The injection of cold water has the remarkable effect of allowing of the production of a high-strength dried product in a single operation because it allows of the use of hot inlet gases without the disadvantages hitherto attendant thereon. Moreover the water, in addition to preventing premature drying and lowering the temperature locally (by absorption of heat due to evaporation), appears to act as a catalyst in the reaction. I may, less desirably, inject steam or use lime containing excess of moisture but I prefer the use of liquid water for the reasons stated.

The quantity of water added is preferably above 0.5% calculated on the weight of the bleaching powder produced, but I prefer to use quantities of the order of 2 to 3%. If precautions are taken to remove dust, (which is necessary owing to the high velocity of the gases) a very much larger quantity of water may be used, with great increase in the speed of the reaction.

With about 2-3% of water, it is possible to make

ordinary bleaching powder of 35-37% available chlorine with an output about 100% more than is possible in the same rotary tube, without water, under otherwise identical conditions. Using less water, a less increase is easily obtained e.g. 30%.

When making so-called "tropical" bleaching powder, it is believed novel to obtain this product in one operation by the use of hot inlet gas. Considerable increases of output are obtained according to the invention though obviously the output of tropical bleaching powder will be less than that of the ordinary product, since it is necessary to chlorinate and dry in one operation.

My object in performing the reaction in presence of an excess of moisture is not to raise the percentage of available chlorine in the final product, (since my product, like other commercial bleaching powders, contains substantially less than the theoretically possible quantity of available chlorine) but to increase the possible rate of reaction by allowing for local dissipation of undesirable heat and probably by catalytic acceleration of the chlorination.

The term "chlorinatable lime" is employed to include both partially and wholly slaked lime and partially chlorinated lime.

We use the term "hot gas" in the claim to refer to gas heated above 50° C. which is often regarded in this art as a temperature which should be avoided, to prevent decomposition of the product.

I declare that what I claim is:—

1. The process of making bleaching powder by circulating a large volume of dilute chlorine in counter current with chlorinatable lime and simultaneously introducing liquid water at the chlorinating zone.

2. The process of making bleaching powder by circulating a large volume of dilute chlorine in counter current with agitated slaked lime and simultaneously introducing a spray of liquid water at the chlorinating zone.

3. The continuous process of producing bleaching powder by chlorinating a solid chlorinatable material which includes the step of injecting liquid water into the reaction zone.

4. In the process of making bleaching powder by circulating a large volume of dilute chlorine in counter current with agitated chlorinatable lime, the step of admitting liquid water to the chlorinating zone in a quantity of at least 2-3% H<sub>2</sub>O of the weight of bleaching powder formed.

5. The process of making tropical bleaching powder by circulating a large volume of hot and substantially dry dilute chlorine in countercurrent with chlorinatable lime agitating the lime and simultaneously introducing liquid water at the chlorination zone.

CHARLES CARTER. 135

65

140

70

145

75

150